

# UNITED STATES PATENT OFFICE.

ALBERT L. CLAPP, OF BRAINTREE, MASSACHUSETTS, ASSIGNOR TO HIDE-ITE LEATHER COMPANY, OF BOSTON, MASSACHUSETTS, A CORPORATION OF MAINE.

## METHOD OR PROCESS OF MAKING LEATHER-BOARD.

1,128,290.

Specification of Letters Patent. Patented Feb. 16, 1915.

No Drawing.

Application filed January 11, 1913. Serial No. 741,477.

To all whom it may concern:

Be it known that I, ALBERT L. CLAPP, a citizen of the United States, residing at Braintree, in the county of Norfolk and State of Massachusetts, have invented certain new and useful Improvements in Methods or Processes of Making Leather-Board, of which the following is a specification.

10 My present invention pertains to an improved method of making leatherboard, the main objects being to remove tannic acid from the stock before the addition of the material employed to waterproof it, where-  
15 by the waterproofing operation is facilitated and the character of the product improved; to conserve such removed tannic acid and other materials that may be in solution; and to utilize such removed material in the  
20 manufacture of the leatherboard.

In the production of waterproof leather-  
board it is necessary in order to insure a  
homogeneous and thoroughly waterproof  
board that the stock should be thoroughly  
25 and evenly, waterproofed throughout, and it  
is likewise desirable that the board should  
contain all the constituent elements of the  
leather scrap from which the board is  
formed. In processes of waterproofing the  
30 stock in which a substance such as a soap  
compound or emulsion, or a solution of  
casein or glue, is mixed with the stock and  
then subjected to the action of a precipitant  
in order to deposit upon the fiber of the  
35 stock an insoluble compound to waterproof  
the same, the presence of tannic acid tends  
to impede proper action, and to cause the  
waterproofing material to coagulate or cur-  
dle, which, of course, is fatal to proper dis-  
40 tribution of the material evenly and thor-  
oughly in and through the stock; and the  
removal of the tannic acid renders the fibers  
of the stock more receptive to the water-  
proofing material.

45 It has heretofore been proposed to re-  
move the free tannic acid, or some portion  
of it, by washing the stock in water. As this  
process has been carried on, however, the  
wash water has been run to waste, and there  
50 has been a waste of the water-soluble in-  
gredients of the leather stock, such ingredi-  
ents passing off with the wash water.

55 My present invention consists in a method  
by which such ingredients may be utilized  
in the process and conserved in the product.

After washing the charge of stock, which, as will be understood, is produced from leather-scrap, the wash water, having been drained off or removed in a suitable manner is conveyed to a storage tank, and after 60 the soap compound or emulsion or other waterproofing agent has been added to the charge in the beater and thoroughly mixed therewith, the water containing the tannic acid is returned to the mixture, where it will 65 act as a precipitant upon the soap or emulsion and cause an insoluble precipitate to be deposited upon the fibers of the stock. Since the tannic acid contained in the wash water from any one charge will hardly be suffi- 70 cient to cause a precipitation of sufficient waterproofing material for the stock, it will in most cases be desirable to add to the water containing the tannic acid alum or some other suitable precipitant in quantities 75 sufficient to complete the precipitation of the waterproofing material. The amount of alum, if any, necessary to be added in order to accomplish the complete precipitation will depend on the quantity of tannic acid 80 which is present in the water and can readily be determined by analysis. It is also desirable to add alum to the water on account of the presence in the water of soluble organic matters in addition to the tannic 85 acid, which matters are insoluble in the presence of alum, and will therefore be precipitated when the alum is added to the water, thus becoming capable of retention in the finished product. The precipitation of these 90 other organic matters is facilitated by heating the water to a temperature above the coagulation point of albumen, say 180° F. If the water is heated, it should, of course, be allowed to cool again before being re- 95 stored to the beater engine.

Having thus described my invention, what I claim is:

1. In the manufacture of leatherboard, the process of washing that portion of the 100 stock consisting of leather scrap or fibers, removing the wash water, mixing with the stock a waterproofing material capable of depositing on the fibers thereof by a reaction with tannic acid an insoluble precipitate, 105 and thereafter adding the wash water to the mixture.

2. In the manufacture of leatherboard, the process of washing that portion of the 110 stock consisting of leather scrap or fibers,

removing the wash water, mixing with the stock a waterproofing material capable of depositing on the fibers thereof by a reaction with tannic acid an insoluble precipitate, 5 and thereafter adding to the mixture the tannic acid contained in the wash water.

3. In the manufacture of leatherboard, the process of washing that portion of the stock consisting of leather scrap or fibers, 10 removing the wash water, mixing with the stock a waterproofing material capable of depositing on the fibers thereof by a reaction with tannic acid an insoluble precipitate, and thereafter using the tannic acid contained in the wash water as a precipitant to react on the waterproofing material. 15

4. In the manufacture of leatherboard, the process of washing that portion of the stock consisting of leather scrap or fibers, 20 removing the wash water, mixing with the stock a waterproofing material capable of

depositing on the fibers thereof by a reaction with tannic acid an insoluble precipitate, adding alum to the wash water, and thereafter adding the wash water to the mixture. 25

5. In the manufacture of leatherboard, the process of washing that portion of the stock consisting of leather scrap or fibers, 30 removing the wash water, mixing with the stock a waterproofing material capable of depositing on the fibers thereof by a reaction with tannic acid an insoluble precipitate, adding alum to the wash water, heating the wash water, and thereafter adding the wash water to the mixture. 35

In testimony whereof I have signed my name to this specification in the presence of two subscribing witnesses.

ALBERT L. CLAPP.

Witnesses:

HORACE A. DODGE,  
BENNETT S. JONES.